

## UNITED STATES PATENT OFFICE.

HYMAN STEIN AND WILLIAM E. AUSTIN, OF NEW YORK, AND IRVING LIEBOWITZ, OF BROOKLYN, NEW YORK, ASSIGNORS TO STEIN FUR DYEING CO., INC., OF NEW YORK, N. Y., A CORPORATION OF NEW YORK.

## METHOD OF FABRICATING FELTS AND FELT MATERIALS.

No Drawing.

Application filed February 10, 1925 Serial No. 8,306.

Our present invention relates to methods of rendering animal fibers and the like, especially fur skins and the like, or the hair obtained from such skins, suitable for felting, and relates also to the felting process itself, particularly in combination with certain steps for bleaching and dyeing the fibers either before, during, or after the steps of the process for rendering the hair or other animal fibers, or the fur skins carrying such hair, suitable for felting. Our invention may be applied with particular success to the treatment of dark-colored animal fibers, particularly dark colored hair and fur skins carrying the same to render the same suitable for the felting operation and to derive from the same a feltable fiber of a light color very suitable for dyeing and for felting into a felted fabric.

Our invention aims to devise methods of the general character described above which are simple to practice, which are economical in the matter of the time, labor, material and equipment required for their practice, and which yield intermediate and end products of superior qualities for the intended purpose. Our invention, so far as the same relates to such products in the various stages of their production, is claimed in a copending application of ours filed of even date herewith and entitled "Felts and felt materials and articles, such as hats and hat bodies, made of the same."

In the accompanying specification we shall describe illustrative embodiments of the processes of the present invention. It is, however, to be clearly understood that our invention is not limited to the specific forms thereof herein described for purposes of illustration only.

Before describing in detail the aforesaid illustrative embodiments of the present invention, it may be desirable briefly to point out certain disadvantages of the prior art so far as the same relates to the field of the present invention. Hitherto it has been proposed, for example, to "carrot" animal fibers, such as fur skins and the like or the hair of such skins, to render the same suitable for felting operations, by treating such skins or the hair of the same with an acid solution of nitrate of mercury. This treatment, if

used by itself for the entire "carrotting" operation, tends to weaken and otherwise hurt the hairs or equivalent fibers.

55

Furthermore, where it is desired to obtain a light colored mass of feltable hairs or other animal fibers, if the hair is bleached first, the bleaching operation generally tends to weaken the hair to such an extent that the subsequent "carrotting" operation, tending further to weaken the hair, would tend often to render the same quite unfit for the subsequent felting operation. It has, therefore, not been feasible to make a light colored mechanically desirable feltable fiber from a dark colored skin by the usual bleaching and "carrotting" operations.

60

On the other hand, if the hair or equivalent animal fibers are first "carroted," as by means of the treatment with the acid solution of nitrate of mercury referred to above, this treatment would tend to render the subsequent bleaching operation imperfect and otherwise quite unsatisfactory. In any event, both the "carrotting" and the bleaching operations as hitherto conducted, in whatever order they have been carried out, would both singly and conjointly tend to considerably weaken and otherwise impair the structure and appearance, as well as the felting qualities, of the fur, hair or other fibers to which the treatments of the prior art might be applied.

75

We have discovered a new method of "carrotting" or treating fur skins, hair and other animal fibers to render the same suitable for subsequent felting operations. Our new "carrotting" process is characterized by the fact that it does not substantially hurt the fur, hair or other fibers treated in accordance with such process. The "carrotting" operation of the present invention may moreover be very effectively combined with a bleaching operation whereby dark colored skins or the hair thereof may be ultimately obtained in a condition ideally suited for felting or already felted in a very light color, in which condition the feltable mass or the felted product is admirably suited for dyeing any light or other suitable color. In one of its forms, in fact, our present invention comprehends a preliminary and partial "carrotting" operation followed by a bleaching

80

85

90

95

100

operation which at the same time completes the "carrotting" operation and thus yields a bleached fiber admirably suited for felting.

Referring now to the aforesaid illustrative 5 embodiments of the methods of the present invention, we take first any suitable fur skin or the hair of such skin, or any other suitable animal fiber which it is desired to convert into a feltable fiber. Preferably we 10 treat a fiber which is dark and which we desire to bleach into a light colored, readily feltable fiber. For example, we may take rabbit skins of a dark color and treat the same with great success in accordance with 15 the principles of the present invention.

It may here be stated that the principles of the present invention may be applied with almost equal success either to the fur skin itself, such as the dark or other colored rabbit skins referred to, or to the hair obtained from such skins. It may also here be stated that in accordance with the principles of the present invention, neither the fur skins nor the hair derived from the same need 25 first be washed or "killed" in an alkaline solution, such as a solution of sodium carbonate. However, in some instances, this washing operation, which ordinarily required from about two to about three hours, 30 may be employed, although we prefer to dispense with the same in most instances.

We now treat the fur skins or the hair of the same, referred to above, preferably the dark or other colored rabbit skins or hair 35 from such skins, with a suitable "carrotting" agent, preferably a metallic compound "carrotting" agent, but preferably only to the point of partial completion of the "carrotting" step. For example, I may treat the fur 40 skins or other animal fibers in accordance with the principles of the present invention with nitrate of mercury, obtained, for example, by the solution of metallic mercury in nitric acid, thus obtaining an acid solution 45 of nitrate of mercury. This treatment is preferably continued only to the point of partial completion of the "carrotting" operation, as by using only one-half, or only two-thirds or three-fourths, or any suitable 50 amount of the acid solution of the nitrate of mercury or equivalent metallic or other "carrotting" agent, short of the amount which would be required for the completion of the "carrotting" operation. This is very desirable, 55 since the subsequent bleaching operation serves, at the same time, to complete the "carrotting" operation, all of which is done in accordance with the principles of the present invention without destruction of the hair or other animal fibers and without 60 in any way impairing their ultimate felting qualities. In fact, the felting qualities of animal fibers treated in accordance with the principles of the present invention are superior 65 to those of ordinary fibers treated in

accordance with the methods hitherto employed for this purpose.

We now treat the partially "carrotted" fibers, prior to the subsequent bleaching and completion of the "carrotting" process, with 70 a protective agent, generally a reducing compound, preferably of mineral origin, such as a ferrous compound, for example, ferrous sulphate. In some way, the reasons for which are at present not understood by us, 75 such protective agent, while permitting the bleaching or decolorizing action to proceed under the action of the bleaching agent with remarkable rapidity, protects the leather of the fur skin and the hair of the same from 80 any destructive or weakening effect of the bleaching agent.

For instance, decolorizing or bleaching of fur skins or the like takes place in accordance with the principles of the present invention under the action of a bleaching agent such as hydrogen peroxide, for example, within a short time, as from about one to about four hours. This is contrasted with the twenty-four to seventy-two hours hitherto required for bleaching fur skins by the methods hitherto commonly employed. At the same time the leather and hair of the skins and the fibers of the hair or other animal fibers bleached in accordance with the 90 principles of the present invention, will be found to be in fine condition, with their strength, texture and lustre substantially unimpaired. At the same time, we have discovered that the "carrotting" operation is 100 completed by what we have thus far termed the "bleaching" operation. It appears that the hydrogen peroxide or equivalent bleaching agent acts as a non-metallic "carrotting" agent to complete the "carrotting" operation 105 only partially completed by the acid solution of nitrate of mercury or equivalent metallic "carrotting" agent.

While we do not wish to be limited to any particular theory or explanation as to why this remarkable, unexpected and commercially valuable result is obtained, our present explanation is that the presence on or in the fibers of the fur skins or the like of the mineral reducing agent or its equivalent, the effectiveness of which appears not to be diminished by the presence of the nitrate of mercury or other metallic "carrotting" agent, prevents too violent an action of the hydrogen peroxide or equivalent bleaching agent. At the same time, the hydrogen peroxide or equivalent bleaching agent acts to complete the "carrotting" operation and the ultimate product is a fiber light in color and remarkably well adapted for subsequent felting operations. In fact, the presence of the metallic protective agent, such as the ferrous compound referred to, or its equivalent, especially in the presence of the nitrate of mercury or equivalent metallic "carrotting" 130

agent, not only protects the leather and the hair of the fur skins or other animal fibers from destructive or weakening action, but at the same time actually accelerates the desired decolorizing or bleaching action and the completion of the "carrotting" operation, so that the combined bleaching and "carrotting" operation take only from about one to about four hours, instead of the twenty-four to seventy-two hours hitherto required for the imperfect or even destructive bleaching methods as hitherto practiced.

Since the protective agent and bleaching accelerator in accordance with the principles of the present invention, generally comprises a reducing agent or compound, preferably of mineral origin, such as a ferrous compound, for example, ferrous sulphate, which would tend to be oxidized more or less readily on exposure to the air, we prefer to add to the protective agent preferably before the same is applied to the fur skin or the like, prior to the bleaching and "carrotting" operation, a stabilizing agent. The purpose of the stabilizing agent is to stabilize the protective agent and to prevent too rapid oxidation or deterioration of the same. Where, as is preferred, ferrous sulphate is used for the protective agent, we prefer to use for the stabilizing agent ammonium chloride. The fur skins or the like, after having been treated with a solution of the protective compound which may or may not contain therein the stabilizing agent, are thereafter subjected to the combined bleaching and "carrotting" operation, after which they may be dyed in any of the light or other shades such as can at the present time be produced only by dyeing natural white or other light colored skins or other animal fibers.

The following is a specific example of one mode of applying the method of the present invention, it being understood, however, that the following description is given merely by way of illustration and that the process is not limited to the specific details of the following illustrative example:

The dark colored rabbit skins, preferably without being first washed or "killed" in an alkaline solution, such as a solution of sodium carbonate, which washing operation ordinarily requires from about two to about three hours, are immersed in an acid solution of nitrate of mercury in an amount sufficient only partially to "carrot" such skins or like animal fibers. For example, only one-half, or even as much as two-thirds or three-fourths, of the usual amount of acid solution of nitrate of mercury is employed so that the "carrotting" operation at this stage is only partially completed.

The partially "carroted" skins or other animal fibers are then rinsed and thoroughly hydro-extracted. The skins are then immersed in a solution of the protective agent,

such as in a solution of ferrous sulphate, and there allowed to remain over night. While the strength of the ferrous sulphate solution or its equivalent may vary within considerable limits, we prefer to use an aqueous solution of ferrous sulphate of a strength of from about 0.5 to about 5.0 per cent of the solid crystallized ferrous sulphate, by weight. Such a solution may or may not contain the stabilizing agent. If a stabilizing agent, such as ammonium chloride, is used, we prefer to use it in an amount approximately proportionate to the amount of ferrous sulphate used and equalling from about 0.5 to about 5.0 per cent of ammonium chloride, by weight.

The fur skins or the like, after having been soaked for from about 8 to about 12 hours in the solution of the protective agent, with or without the addition of the stabilizing agent, are then rinsed and hydro-extracted. The treatment apparently impregnates or fills the voids and interstices of the fibers with the solution of protective agent. The fur skins thus treated are now immersed in a solution of hydrogen peroxide or equivalent bleaching agent. However, in place of hydrogen peroxide, we may use other bleaching agents, particularly sodium peroxide or sodium perborate, which yield hydrogen peroxide in solution in the presence of certain liberating agents, generally of an acid character. The amount of hydrogen peroxide used may vary from about five (5.0) to about one hundred (100.0) per cent by volume of a three (3.0) per cent solution of hydrogen peroxide. We prefer that the temperature at which the bleaching or decolorizing operation is carried out shall be between 60° and 100° F.

The skins or hair are subjected to the action of the bleaching and "carrotting" agent until they have been sufficiently decolorized. The bleached and now completely "carroted" skins are then rinsed and can, if desired, be dyed directly in accordance with any of the well-known or desirable processes employed for dyeing furs or the like. We may, however, subject the bleached or decolorized skins or hair to the usual dyeing operation of washing and mordanting, and then dyeing the washed and mordanted skins or hair in accordance with the practice hitherto generally employed for dyeing furs and hair.

It may here be stated that a metallic salt or salts may be added to the solution of the protective agent, with or without the stabilizing agent, provided such metallic salt or salts are compatible with the ferrous sulphate or equivalent protective agent. In such a case, the combined decolorizing and "carrotting" process proceeds in exactly the same way as before, while the additional salt or salts may act a mordant for the sub-

sequent dyeing process where a mordant is desired or needed for this purpose. It may here also be stated that while, in accordance with our experience up to the present time, 5 the foregoing process may be successfully applied to all dark colored furs, the concentration of the reagents employed and the methods of subjecting the fur skins and the like to the various partial carroting, protective, and combined bleaching and "carroting" operations, as well as the subsequent mordanting and dyeing operations, will depend very largely upon the nature of the skins or other animal fibers being treated, 10 the factors of temperature, concentrations, lengths of time of treatment, and the like, or any particular kind of animal fiber or the like, being readily determined by trial and experiment.

20 It may here be stated that in addition to the mineral protective agent, such as the ferrous sulphate, with or without the addition of the stabilizing agent, the solution for giving the fur skins or the like their protective treatment for the subsequent combined bleaching and "carroting" operation may contain other compatible metal salts, as well as suitable protective colloids, such as glue, gelatin, or the like, generally in 25 relatively small amounts. It may here also be stated that the methods described above may be applied with almost equal success in the treatment of skins which have already 30 been dyed, either a dark or a light color, and whether satisfactorily or not, but preferably skins which have been dyed by the use of a mordant consisting of a ferrous compound, such as ferrous sulphate, or an equivalent substance, thus producing from 35 the previously dyed skins and hair the superior products described above.

The advantages of the foregoing embodiments of the processes of the present invention are numerous and of great practical 45 importance and may be briefly summarized as follows: In the first place the foregoing embodiments of the present invention enable the "carroting" operation to be economically and quickly effected, with little weakening of the fibers, while yielding fibers which are 50 readily feltable and which may be compacted to yield a remarkably fine felt, both as to texture, strength and color. Especially where dark colored hair or other fibers 55 are employed, the process enables a feltable mass of fibers to be obtained from such dark colored skins or hair in a very light color ordinarily obtainable only by the treatment of naturally white or light colored 60 skins or hair derived from the same. By combining the bleaching operation with the completion of the "carroting" operation, as above described, a ready control of the "carroting" operation and of the bleaching 65 operation is rendered possible and a final

product obtained which is remarkable for its strength, texture, and felting qualities. The use of the ferrous or other mineral protective agent or its equivalent not only accelerates the bleaching operation but also 70 seems to improve the "carroting" operation and to yield a readily feltable fiber of remarkable strength and fineness of texture.

It may here be stated that under certain conditions the combined bleaching and "carroting" operation by means of a non-metallic "carroting" agent may be carried out first, after which the "carroting" operation may be completed by regulating the amount and length of time of treatment 80 with the acid solution of nitrate of mercury or its equivalent. It may here also be stated that the bleaching operation may be carried out with complete success on fibers or even felts already completely "carroted" by treatment with an acid solution of nitrate of mercury, or equivalent reagent. In fact, the bleaching operation may be carried out with remarkable success on shaped felted bodies such as hat bodies, after the "carroting" operation has been completed. Or else such fibers, masses of felt, or shaped felted bodies, may first be bleached and partially carroted and thereafter "carroted" to completion as already indicated above. Other 90 advantages of the methods of the present invention will readily occur to those skilled in the art to which the present invention relates.

What we claim as our invention is:

1. The method of treating animal fibres and the like to render the same more suitable for felting operations, which comprises treating such fibres with a metallic compound carroting agent and with a protective agent comprising a ferrous salt to protect such fibres against 105 excess action thereon by a subsequent bleaching agent.

2. The method of treating animal fibres and the like to render the same more suitable 110 for felting operations, which comprises treating such fibres with a carroting agent and with a protective agent in the form of a ferrous salt to protect such fibres against 115 excess action thereon by a subsequent bleaching agent.

3. The method of treating animal fibres and the like to render the same more suitable for felting operations, which comprises treating such fibres with a mercurial carroting 120 agent and with a protective agent comprising a ferrous salt to protect such fibres against excess action thereon by a subsequent bleaching agent.

4. The method of treating animal fibres, 125 such as fur skins, hair and the like, to render the same more suitable for felting operations, which comprises treating such fibres with a metallic compound carroting agent and with a non-metallic carroting agent.

5. The method of treating animal fibres, such as fur skins, hair and the like, to render the same more suitable for felting operations, which comprises treating such fibres with a 5 mercurial carroting agent and with a non-metallic carroting agent. thereafter treating such fibres with a non-metallic carroting agent in the presence of a protective and accelerating agent to protect such fibres against excess action thereon by said non-metallic carroting agent. 70
6. The method of treating animal fibres, such as fur skins, hair and the like, to render the same more suitable for felting operations, 10 which comprises treating such fibres with a metallic compound carroting agent and thereafter treating such fibres with a non-metallic carroting agent. 75
7. The method of treating animal fibres, 15 such as fur skins, hair and the like, to render the same more suitable for felting operations, which comprises treating such fibres with a mercurial carroting agent and thereafter treating such fibres with a non-metallic carroting agent. 80
8. The method of treating animal fibres, such as fur skins, hair and the like, to render the same more suitable for felting operations, which comprises treating such fibres with a 25 mercurial carroting agent and with a non-metallic carroting agent comprising hydrogen peroxide. 85
9. The method of treating animal fibres, such as fur skins, hair and the like, to render the same more suitable for felting operations, 30 which comprises treating such fibres with a metallic compound carroting agent and with a non-metallic carroting agent comprising hydrogen peroxide. 90
- 35 10. The method of treating animal fibres, such as fur skins, hair and the like, to render the same more suitable for felting operations, which comprises treating such fibres with a mercurial carroting agent and thereafter treating such fibres with a non-metallic carroting agent comprising hydrogen peroxide. 95
- 40 11. The method of treating animal fibres, such as fur skins, hair and the like, to render the same more suitable for felting operations, 100 which comprises treating such fibres with a metallic compound carroting agent, and with a non-metallic carroting agent in the presence of a protective and accelerating agent to protect such fibres against excess action thereon by said non-metallic carroting agent. 105
- 45 12. The method of treating animal fibres, such as fur skins, hair and the like, to render the same more suitable for felting operations, 110 which comprises treating such fibres with a mercurial carroting agent, and with a non-metallic carroting agent in the presence of a protective and accelerating agent to protect such fibres against excess action thereon by the hydrogen peroxide. 115
- 50 13. The method of treating animal fibres, such as fur skins, hair and the like, to render the same more suitable for felting operations, 120 which comprises treating such fibres with a metallic carroting agent, and with hydrogen peroxide in the presence of a protective and accelerating agent to protect such fibres against excess action thereon by the hydrogen peroxide. 125
- 55 14. The method of treating animal fibres, such as fur skins, hair and the like, to render the same more suitable for felting operations, 130 which comprises treating such fibres with a mercurial carroting agent, and with hydrogen peroxide in the presence of a protective and accelerating agent to protect such fibres against excess action thereon by the hydrogen peroxide.
- 60 15. The method of treating animal fibres, such as fur skins, hair and the like, to render the same more suitable for felting operations, which comprises treating such fibres with a metallic compound carroting agent, and with hydrogen peroxide in the presence of a protective and accelerating agent to protect such fibres against excess action thereon by the hydrogen peroxide. 135

tions, which comprises treating such fibres with a metallic carroting agent, and with a metallic compound carroting agent, and with a non-metallic carroting agent in the presence of a metallic protective and accelerating agent comprising a ferrous salt to protect such fibres against excess action thereon by said non-metallic carroting agent.

21. The method of treating animal fibres, such as fur skins, hair and the like, to render the same more suitable for felting operations, which comprises treating such fibres with a mercurial carroting agent, and with a non-metallic compound carroting agent in the presence of a metallic compound protective and accelerating agent comprising a ferrous salt to protect such fibres against excess action thereon by said non-metallic carroting agent.

22. The method of treating animal fibres, such as fur skins, hair and the like, to render the same more suitable for felting operations, which comprises treating such fibres

with a metallic carroting agent, and with hydrogen peroxide in the presence of a metallic protective and accelerating agent comprising a ferrous salt to protect such fibres against excess action thereon by the hydrogen peroxide.

23. The method of treating animal fibres, such as fur skins, hair and the like, to render the same more suitable for felting operations, which comprises treating such fibres with a mercurial carroting agent, and with hydrogen peroxide in the presence of a metallic compound protective and accelerating agent comprising a ferrous salt to protect such fibres against excess action thereon by the hydrogen peroxide.

In testimony whereof, we have signed our names to this specification this 29th day of January, 1925.

HYMAN STEIN.  
IRVING LIEBOWITZ.  
WILLIAM E. AUSTIN.